

## UNITED STATES PATENT OFFICE

2,114,028

## INSULATING COMPOUND

Harold F. Ormerod, Yonkers, N. Y., assignor to  
 Anaconda Wire & Cable Company, New York,  
 N. Y., a corporation of Delaware

No Drawing. Application May 28, 1936,  
 Serial No. 82,260

4 Claims. (Cl. 106—12)

This invention relates to insulating composition for use in filling electrical apparatus subjected to high tension electric currents or stresses, and particularly for filling such equipment as 5 potheads and other terminals. This application is a continuation-in-part of my copending application Serial No. 738,815, filed August 7, 1934.

In terminating a high tension cable, where it enters a power station or sub-station, or is 10 connected to electrical apparatus, the cable is extended into a connecting apparatus of suitable construction where it is connected to electrical apparatus, bus-bars, or other equipment. One type of connecting device is what is known as a 15 pothead consisting of a metal body with a hollow porcelain insulating cover, through which the conductor is passed to an overhead connection outside of the pothead.

After entering the pothead, the cable is generally stripped, or partially stripped, of its wrapping of impregnated insulation, and to supply 20 the necessary insulation between the metal body and the conductor, the pothead is filled with an insulating composition, generally an asphalt, or 25 similar material. Another type of terminal structure is a junction box generally made of metal and containing bus-bars and lateral connecting cables. These junction boxes may also be filled with an insulating composition to protect any 30 exposed conductors from moisture or from grounding.

Cable splices and other constructions are also used at the terminals for cables.

Wherever apparatus of the above type has been 35 filled with an insulating medium, it has usually been the practice to use asphalt, or similar bituminous material either plain or compounded with other liquefiable ingredients. The asphalt has generally been filled into the pothead, or other 40 metal container by melting it and pouring it into the container, permitting it to set therein.

Asphalts and compounds of like nature, which have heretofore been used have, in general, supplied a high dielectric strength, but they suffered 45 from the disadvantage that they have a high specific inductive capacity, generally higher than that of the insulation of the cable. Therefore, they tend to become overstressed in service. This is overcome to some extent by partially or fully 50 insulating the exposed portion of the conductor within the pothead or terminal body by wrapping these exposed parts with tapes which requires a hand operation.

Moreover, the asphalt type of filling compound 55 must be melted in order to be poured into

the terminal body, usually through a small opening, thereby having a tendency to include condensate and air in the filling and cause electrical leakage and, eventually, failure. An obstacle also arises to filling certain forms of potheads or 5 chambers owing to the tendency for the asphalt to rapidly chill and solidify before it can enter and fill the narrower passages. Also these asphalt compounds have a tendency to shrink when solidified, leaving voids which are sources of 10 weakness and points of potential failure.

An object of my present invention is to provide an improved filling composition for electrical apparatus, such as potheads and terminal structures, which will have the required dielectric strength without an abnormally high specific 15 inductive capacity and which is of such a consistency as readily to fill the potheads or other structures and to avoid the formation of voids, etc.

The filling material of my invention comprises 20 a pasty, pulpy composition of fibrous insulating material such as paper pulp and insulating liquid such as mineral oil or composition of mineral and other oil, such as resin oil, impregnating and filling the pulp. The fibres are in a free substantially 25 unmatted condition and may be molded or packed into spaces to be filled, and the oil is in sufficient quantity to fill the interstices and spaces within the fibrous mass.

For impregnating a paper insulated cable, a mineral oil or a mixture of abietic acid and oil is commonly used and the same liquid insulation 30 is suitable for forming the compound of my invention. In general, however, any impregnating insulating fluid used in the cable itself will be satisfactory as the filling or impregnating fluid of my invention.

The fibrous material may be in the form of a loose fluff of fibres having about the size and 40 characteristics of a loosely fluffed paper pulp so that the resulting pasty composition of insulating fluid or liquid and pulp may be readily filled or pressed into the pothead or other container in which it is to be used. The quantity of pulp in 45 the composition may be varied to give a resulting composition having a desired fluidity and may be governed to some extent by the particular oil or insulating fluid being used and by the fibre density or coarseness of the fibres used. 50 Generally, the maximum quantity of paper pulp to be used with an oil of the type commonly used for impregnating a paper wrapped cable will be about 25% dry weight.

Smaller percentages, such as about 10% will, 55

in general, be a desirable proportion to use with the usual type of paper pulp.

As the composition is generally a pasty or pulpy mass, it may be readily filled into the containers and compacted therein and is not subject to the formation of cracks, such as may happen upon the cooling of solid or rigid filling material.

The pulp of fibrous material holds the liquid in a fibrous network so that it does not readily 10 flow out of position. The fluidity of the oil is thereby checked. The mass of the pulp retains its ability to move and to alter its shape when pressed into position.

The pulp and liquid insulating composition of 15 the above invention has the advantage that its dielectric properties closely approximate those of the impregnated paper wrapping of the cable itself. This is undoubtedly due to the breaking up of the dielectric paths by the fibres of the 20 paper and in this way the dielectric properties are increased over those of the insulating liquid itself.

Through the above invention, a sudden change 25 in the specific inductive capacity from the cable insulation to the filling composition within the terminal body is reduced to a minimum or entirely eliminated. By the proper combination of pulp and insulating fluid, the dielectric strength of the filler compound in a direction radially of 30 the conductor can be made equal to or higher than the strength of the cable insulation. Moreover, the dielectric strength of the filler composition in an axial direction will be of the same order as the radial strength because of the fact

that there is no separating line, such as may be caused by the gelling of a liquefiable solid compound on either the terminal body walls, or the surface of the conductor.

Through the above invention, I have, therefore, 5 provided a filling composition of wide general use for insulating an electrical conductor from a surrounding spaced enclosing structure.

What I claim is:

1. A pasty filling composition consisting of a 10 cable insulating oil and a fibrous pulp of non-conducting material immersed in said oil and being not over about 25% of the weight of the composition and the resulting mixture being fluid.

2. A pasty filling composition consisting of a 15 cable insulating oil composition and paper pulp immersed therein, the paper pulp constituting not over about 25% of the total weight of the composition and the resulting mixture being fluid.

3. A pasty filling composition consisting of a 20 cable insulating oil of low specific inductive capacity and a fibrous pulp of non-conducting material immersed in said oil and constituting not over about 25% of said composition and the 25 resulting mixture being fluid.

4. A pasty filling composition consisting of a 30 pulp of non-conducting fibrous material and an insulating fluid consisting of a mineral oil and abietic acid penetrating and saturating said pulp, said pulp comprising not over about 25% by weight of said composition and the resulting mixture being fluid.

HAROLD F. ORMEROD.